

1

3,403,025

**DESENSITIZATION OF SILVER HALIDES  
TO VISIBLE RADIATION WITH THIURAM DISULFIDES**

William W. Rees and William H. Russell, Rochester, N.Y., assignors to Eastman Kodak Company, Rochester, N.Y., a corporation of New Jersey  
No Drawing. Filed Aug. 25, 1965, Ser. No. 482,632  
20 Claims. (Cl. 96—101)

**ABSTRACT OF THE DISCLOSURE**

The photographic sensitivity of silver halides to visible radiation with a combination of a thiuram disulfide silver halide desensitizer and a piazine is disclosed. X-ray sensitive materials employing such silver halides exhibit improved room-light handling characteristics.

This invention relates to reducing the sensitivity of silver halides to visible radiation and compositions which are useful for this purpose. In one of its aspects, this invention relates to photographic silver halide emulsions and elements which can be used in radiography. In another of its aspects, this invention relates to X-ray sensitive photographic elements which have materially reduced sensitivity to visible radiation.

It is known that photographic silver halides, particularly those employed in photographic silver halide emulsions designed for use in radiography, can be substantially desensitized to visible radiation without substantially affecting their sensitivity to X-rays. For example, U.S. Patent 3,184,313, issued May 18, 1965, discloses the use of thiuram disulfides to reduce the sensitivity of photographic silver halide emulsions to visible radiation. The thiuram disulfide silver halide desensitizers have the advantage of only slightly lowering the sensitivity of X-ray sensitive elements to X-rays while materially reducing their sensitivity to visible radiation. X-ray sensitive elements containing these thiuram disulfides can be easily handled under ordinary safelight conditions while dry. However, X-ray sensitive elements containing thiuram disulfides are not completely protected against visible radiation while wet, i.e., during processing. It is evident that it would be desirable to protect X-ray sensitive elements against the adverse effects of visible light during all stages of handling, i.e., in both dry and wet stages.

Accordingly, it is an object of this invention to provide a composition which materially reduces the sensitivity of silver halides to visible radiation.

It is another object of this invention to provide X-ray sensitive elements which are stabilized against the effects of visible radiation during both dry and wet handling of the element.

It is another object of this invention to provide a photographic silver halide emulsion which is desensitized to visible radiation without any substantial reduction in sensitivity to X-rays.

It is a further object of this invention to provide an X-ray sensitive photographic element which combines good X-ray speed stability during storage with good stability against the effects of visible radiation during both dry and wet handling.

It is another object of this invention to provide a combination of desensitizing materials which will materially reduce the sensitivity of silver halides to visible radiation without adversely affecting sensitivity to X-rays.

It is another object of this invention to provide photographic silver halide emulsions and elements which contain a combination of a thiuram disulfide and a piazine which combination materially reduces the photographic

2

sensitivity of photographic silver halides to visible radiation without adversely affecting their sensitivity to X-rays.

Other objects of this invention will be apparent from an examination of the specification and claims which follow.

In accordance with this invention it has been found that a combination comprising a thiuram disulfide and a piazine containing a pyrazine ring to which two 6-membered carbocyclic rings are fused symmetrically will materially reduce the sensitivity of photographic silver halides to visible radiation without any substantial adverse effect on X-ray sensitivity.

In one embodiment of this invention, the aforementioned combination is employed to desensitize a photographic silver halide emulsion to visible radiation. Another embodiment of this invention relates to a photographic element comprising a support and a photographic silver halide layer desensitized to visible radiation with a combination of a thiuram disulfide silver halide desensitizer and a piazine containing a pyrazine ring to which two 6-membered carbocyclic rings are fused symmetrically.

A significant feature of this invention is that the thiuram disulfide silver halide desensitizer and the piazine must be used in combination to protect X-ray sensitive materials from the adverse effects of visible radiation during all stages of handling, i.e., in the dry and wet stages, and also to stabilize the X-ray speed of the element during storage. Thus, as shown in the following working examples, the thiuram disulfides are effective to stabilize the speed and fog of a silver halide emulsion during dry handling but they do not give good X-ray speed stability during storage. Conversely, the piazine imparts good wet stability but gives very poor incubation speed stability.

The disulfide compounds employed in the practice of this invention are thiuram disulfide silver halide desensitizers. Typical thiuram disulfide silver halide desensitizers are disclosed in U.S. Patent 3,184,313, issued May 18, 1965. These compounds are characterized by marked desensitizing action toward silver halide emulsions insofar as their sensitivity to visible radiation is concerned (particularly in the blue region of the spectrum) while retaining substantially the sensitivity of the emulsions to X-rays. The concentration of thiuram disulfide silver halide desensitizer employed is subject to wide variation depending upon the particular silver halide used, the amount of gelatin or other colloidal binder and other variables. In general, quite useful results can be obtained at concentrations as low as 2 mg. per mole of silver halide, while concentrations as high as 75 mg. per mole of silver halide can be used without adversely affecting the X-ray sensitivity too seriously. The preferred range of thiuram disulfide employed in the practice of this invention is in the range of about 20 to about 30 mg. of thiuram disulfide per mole of silver halide. As already indicated, silver halide desensitizers are employed in combination with the piazines described herein. While the concentration of the thiuram disulfide and the piazine in the combination can be widely varied, it is preferred that the major component of the combination be thiuram disulfide, useful results being obtained with combinations in which the weight ratio of thiuram disulfide to piazine is in the range of about 2:1 to about 20:1, preferably about 2:1 to about 10:1. Typical thiuram disulfide desensitizers which can be employed in the practice of this invention include those represented by the following general formula:



70 wherein R and R<sub>1</sub> each represents an alkyl group, such as methyl, ethyl, propyl, butyl isobutyl, etc. (e.g., an alkyl



**5**

2,3-diaminophenazine



3-amino-2-hydroxyphenazine



3,6-diaminophenazine



3-amino-7-dimethylaminophenazine



2-methyl-3-amino-7-dimethylaminophenazine



naphtho-phenazine



naphthazine



phenanthrophenazine



2,3-dihydroxyphenazine

**6**

2-acetamino-3-acetoxyphenazine



1,3-diamino-5-methylphenazinium chloride



1,3-diamino-5-phenylphenazinium chloride



3,7-diamino-5-phenylphenazinium chloride



2,8-dimethyl-3,7-diamino-5-phenylphenazinium chloride



3-amino-7-phenylamino-5-phenylphenazinium chloride



2,3,7,8-phenylamino-5-phenylphenazinium chloride



1,3-diamino-5-ethylphenazinium chloride



## 1,3-diamino-5-p-hydroxyethylphenazinium chloride



## 1,3-diamino-5-benzylphenazinium chloride



The desensitizing combination of this invention can be used to materially reduce the sensitivity to visible radiation of any of the different types of photographic silver halides. For example, silver halides such as silver chloride, silver bromide, silver chlorobromide, and the like can be employed in practicing this invention although iodide containing photographic silver halide emulsions are especially useful. Such emulsions include silver bromoiodide, silver chloroiodide, silver chlorobromide and the like. Photographic silver halide emulsions which form the latent image predominantly within the silver halide grain can be usefully employed in the practice of this invention. Such internal latent image emulsions are described in Davey and Knott U.S. Patent 2,592,250 issued Apr. 8, 1952.

The photographic silver halides desensitized according to the practice of this invention can be dispersed in any of the conventional hydrophilic water permeable binding materials, particularly those employed in the preparation of photographic silver halide emulsions and elements, as exemplified by gelatin, colloidal albumin, cellulose derivatives, synthetic resins such as polyvinyl compounds, acrylamide polymers and the like as well as mixtures of these materials. Such binding materials are generally employed in coating photographic silver halides on supports. However, photographic silver halides which are coated in the absence of such binding materials, for example, those coated by vacuum deposition, can be readily desensitized according to the practice of this invention.

The photographic silver halides employed in the practice of this invention can be coated on a wide variety of supports in preparing photographic elements. The silver halides can be coated on one or both sides of the support, which is preferably transparent and flexible. Typical supports are cellulose nitrate film, cellulose ester film, polyvinyl acetal film, polystyrene film, polyethylene terephthalate film, and related films or resinous materials as well as glass, paper, metal and the like. Supports such as paper which are coated with  $\alpha$ -olefin polymers, particularly polymers of  $\alpha$ -olefins containing two or more carbon atoms, as exemplified by polyethylene, polypropylene, ethylene-butene copolymers and the like, can also be employed.

In order to decrease still further the sensitivity of the silver halide emulsions of our invention to visible radiation, a small amount of a light-absorbing organic dye can be employed either in the emulsion or in an overcoating layer. Since the silver halide emulsions of our invention may retain some sensitivity in the blue region of the spectrum, it has been found that many azo dyes, such as tartrazine, can be usefully employed. Other visible radiation absorbing dyes which can be employed in such ar-

rangements are 2-(2'-methoxy styryl) quinoline hydrochloride, the condensation product of two molecular proportions of quinaldine methosulfate and one molecular proportion of 4,4-diphenyl dialdehyde pyridine, 4,4'-5 methenyl - bis - (1 - naphthyl-3-methylpyrazoline-5), etc. Other light-absorbing dyes are described in Dostes and Pfaff U.S. application Ser. No. 83,709, filed Jan. 19, 1961. The amount of light-absorbing dye used to reduce the sensitivity of our photographic elements can vary as described in said U.S. application Ser. No. 83,709. Instead of using a dyed silver halide emulsion layer or a dyed overcoating layer to protect further the radiographic sensitive layer, it is possible to use a light-absorbing silver halide emulsion layer which has very low sensitivity to visible radiation. Lippmann-type emulsions can conveniently be employed for this purpose. Silver iodide-containing emulsion layers are also useful for this purpose.

The photographic silver halide emulsions described herein can be chemically sensitized with compounds of 20 the sulfur group, noble metal salts such as gold salts, reduction sensitized with reducing agents, and combinations of these. Furthermore, emulsion layers and other layers present in photographic elements made according to this invention can be hardened with any suitable hardener such as aldehyde hardeners, aziridine hardeners, 25 hardeners which are derivatives of dioxane, oxypoly-saccharides such as oxystarch, oxy plant gums, and the like.

The photographic silver halide emulsions can also contain additional additives, particularly those known to be 30 beneficial in photographic emulsions, including, for example, stabilizers or antifoggants, particularly the water soluble inorganic acid salts of cadmium, cobalt, manganese and zinc as disclosed in U.S. Patent 2,829,404, the 35 substituted triazaindolizines as disclosed in U.S. Patents 2,444,605 and 2,444,607, speed increasing materials, plasticizers and the like. Sensitizers which give particularly good results in photographic compositions are the alkylene oxide polymers which can be employed alone or in 40 combination with other materials, such as quaternary ammonium salts, as disclosed in U.S. Patent 2,886,437 or with mercury compounds and nitrogen containing compounds, as disclosed in U.S. Patent 2,751,299.

This invention can be further illustrated by the following examples of preferred embodiments thereof although 45 it will be understood that these examples are included merely for purposes of illustration and are not intended to limit the scope of the invention unless otherwise specifically indicated.

50

## EXAMPLE 1

As already indicated, the thiuram disulfides or piazines alone, will not combine good X-ray speed stability during 55 storage with protection against visible radiation during both wet and dry handling. To illustrate, an ordinary coarse-grained silver bromoiodide emulsion of the type normally used in radiography, which is chemically sensitized to its optimum speed, is divided into three portions. One portion of emulsion is untreated and serves 60 as a control. Another portion, A, is treated with 22.5 mg. of bis(dimethylthiocarbamyl) disulfide per mole of silver halide. The remaining portion, B, is treated with 20 mg. of 1,3-diamino-5-methylphenazinium chloride per mole of silver halide.

Each of the three portions of emulsion is coated on an 65 ordinary cellulose acetate film support and the coatings are dried. The coatings are then divided into five samples, each of which is tested in the following manner:

Test 1.—Exposure to 80 kv. X-rays. Processed for 6 minutes in an ordinary MQ developer, i.e., a developer 70 containing hydroquinone and N-methyl-p-aminophenol sulfate, such as Kodak Developer D-19b to which is added a small concentration of alkali to increase the pH to about 11.0. After development, the samples are fixed, 75 washed and dried in the usual manner. The speeds of the

samples are measured at a density of 0.85 above fog, the initial control speed being taken as 100 in each case.

Test 2.—A low-intensity light exposure of 60 seconds in an intensity scale sensitometer to a 500-watt bulb modulated with a 2.27 neutral density filter. Processed as described in Test 1.

Test 3.—The samples are incubated for 2 weeks at 120° F., 50% relative humidity before exposure and processing as described in Test 2.

Test 4.—Dry safelight test. This test consists of exposure of the dry element to a safelight containing a 25-watt bulb modulated by a Morlite Filter I-11814 (described hereinafter) for 16 minutes at a distance of two feet from the film plane. Processing is as described in Test 1.

Test 5.—Wet safelight test. This test consists of exposure of the element while immersed in Kodak Developer D-19b to a safelight containing a 25-watt bulb modulated by a Morlite Filter I-11814 for three minutes in a white tray at a distance of two feet from the film plane. After development the samples are fixed, washed and dried in the usual manner.

of the type normally used in radiography, but having a greater sensitivity than the emulsion described in Example 1, is prepared and divided into eight portions. These portions of emulsion are then treated as described below:

| Portion | Treatment                                                                                                                                                       |
|---------|-----------------------------------------------------------------------------------------------------------------------------------------------------------------|
| I       | No further treatment. Control.                                                                                                                                  |
| II      | 20 mg. 1,3-diamino-5-methylphenazinium chloride per mole of silver halide.                                                                                      |
| III     | 30.6 mg. of bis(morpholinothiocarbamyl) disulfide per mole of silver halide.                                                                                    |
| IV      | 30.6 mg. of bis(morpholinothiocarbamyl) disulfide per mole of silver plus 2.0 mg. of 1,3-diamino-5-methylphenazinium chloride per mole of silver halide.        |
| V       | 30.6 mg. of bis(morpholinothiocarbamyl) disulfide per mole of silver halide plus 4.0 mg. of 1,3-diamino-5-methylphenazinium chloride per mole of silver halide. |
| VI      | 30.6 mg. of bis(morpholinothiocarbamyl) disulfide per mole of silver halide plus 2.0 mg.                                                                        |

| Portion | Test 1 |      | Test 2 |      | Test 3 |      | Test 4,<br>gross<br>density | Test 5,<br>gross<br>density |
|---------|--------|------|--------|------|--------|------|-----------------------------|-----------------------------|
|         | Speed  | Fog  | Speed  | Fog  | Speed  | Fog  |                             |                             |
| Control | 100    | 0.07 | 100    | 0.14 | 166    | 0.16 | 2.70                        | 1.54                        |
| A       | 67     | 0.04 | 2.4    | 0.14 | 4.8    | 0.14 | 0.14                        | 0.39                        |
| B       | 76     | 0.02 | 4.4    | 0.14 | 18.0   | 0.14 | 0.15                        | 0.16                        |

<sup>1</sup> Base density=0.13.

### EXAMPLE 2

The combination of thiram disulfides and piazines described herein impart to photographic silver halide elements and emulsions good X-ray speed stability upon storage and protection against visible radiation during both wet and dry handling. To illustrate, several additional coatings similar to Portion A described in Example 1 are prepared. One portion remains unchanged to serve as a control. Three other portions are treated with the varying concentrations of the piazines identified below. The coatings are exposed and processed as described in Tests 1-5 listed in Example 1 to give the following results:

35      VII     30.6 mg. of bis(morpholinothiocarbamyl) disulfide per mole of silver halide plus 4.0 mg. of 1,3-diamino-5-ethylphenazinium chloride per mole of silver halide.

40      VIII    30.6 mg. of bis(morpholinothiocarbamyl) disulfide per mole of silver halide plus 8.0 mg. of 1,3-diamino-5-ethylphenazinium chloride per mole of silver halide.

45      Samples of each of the above emulsions are coated on an ordinary cellulose acetate film support and the coatings

| Addenda (mg./mole-silver halide)                            | Test 1 |     | Test 2 |     | Test 3 |     | Test 4,<br>gross<br>density <sup>1</sup> | Test 5,<br>gross<br>density <sup>1</sup> |
|-------------------------------------------------------------|--------|-----|--------|-----|--------|-----|------------------------------------------|------------------------------------------|
|                                                             | Speed  | Fog | Speed  | Fog | Speed  | Fog |                                          |                                          |
| Control                                                     | 100    | .02 | 100    | .12 | 182    | .12 | 0.14                                     | 0.40                                     |
| Control+1,3-diamino-5-methyl phenazinium chloride (4.0 mg.) | 102    | .02 | 95     | .12 | 191    | .12 | 0.14                                     | 0.32                                     |
| Control+1,3-diamino-5-methyl phenazinium chloride (8.0 mg.) | 107    | .02 | 95     | .12 | 191    | .12 | 0.14                                     | 0.17                                     |

<sup>1</sup> Base density=0.13.

Similar results are obtained when bis(dimethylthiocarbamyl) disulfide is replaced in the above procedure with bis(diisobutylthiocarbamyl) disulfide, bis(1-piperidylthiocarbonyl) disulfide, bis(diethylthiocarbamyl) disulfide, bis(N-methyl-N-phenylthiocarbamyl) disulfide and bis(diphenylthiocarbamyl) disulfide. Other piazines such as phenazine, 2-hydroxyphenazine, 2,3-diaminophenazine, 3-amino-2-hydroxyphenazine, 3,6-diaminophenazine, 1,3-diamino-5-phenylphenazinium chloride, 3,7-diamino-5-phenylphenazinium chloride, 2,8-dimethyl-3,7-diamino-5-phenylphenazinium chloride, 3-amino-7-phenylamino-5-phenylphenazinium chloride and 2,3,7,8-phenylamino-5-phenylphenazinium chloride can also be employed in the above procedure to obtain similar results.

60      exposed and processed as described in Tests 1-5 of Example 1. The following results are obtained:

| Portion     | Test 1,<br>speed | Test 2,<br>speed | Test 3,<br>speed | Test 4,<br>gross<br>density <sup>1</sup> | Test 5,<br>gross<br>density <sup>1</sup> |
|-------------|------------------|------------------|------------------|------------------------------------------|------------------------------------------|
| I (Control) | 100              | 100              | 135              | >4.00                                    | 1.10                                     |
| II          | 82               | 8.0              | 19.0             | 0.53                                     | 0.25                                     |
| III         | 83               | 4.6              | 5.0              | 0.14                                     | 0.25                                     |
| IV          | 94               | 5.8              | 5.8              | 0.14                                     | 0.17                                     |
| V           | 105              | 4.6              | 5.8              | 0.14                                     | 0.15                                     |
| VI          | 97               | 6.0              | 5.5              | 0.14                                     | 0.22                                     |
| VII         | 94               | 5.0              | 5.8              | 9.14                                     | 0.18                                     |
| VIII        | 94               | 5.5              | 5.8              | 9.14                                     | 0.16                                     |

<sup>1</sup> Base density=0.13.

70      It can be seen from the above results that the combinations of this invention give the desired safelight protection, both wet and dry, accompanied by excellent incubation stability and an X-ray sensitivity.

### EXAMPLE 3

An ordinary coarse-grain silver bromoiodide emulsion

Kodak Developer D-19b has the following composition:

|                                | Grams |
|--------------------------------|-------|
| N-methyl-p-aminophenol sulfate | 2.2   |
| Hydroquinone                   | 8.8   |
| Sodium sulfate anhydrous       | 72.0  |
| Sodium carbonate crystalline   | 130.0 |
| Potassium bromide              | 4.0   |
| Water to make 1 liter.         |       |

For use in the present invention, this developer is found most effective when the pH is raised slightly to 11.0 by the addition of additional alkali.

The Morlite I-11814 Safelight Filter transmits visible radiation principally between about 540 and 700 m $\mu$  with maximum transmission at from about 580 to 700 (density of about 0.1 in this range).

Thus, by the practice of this invention there is provided a means for reducing the sensitivity of silver halides to visible radiation without deleteriously affecting their sensitivity to X-rays. This invention makes it possible to protect X-ray sensitive elements from the adverse effects of visible radiation in all stages of processing, i.e., in both the dry and wet stages.

Although the invention has been described in considerable detail with reference to certain preferred embodiments thereof it will be understood that variations and modifications can be effected without departing from the spirit and scope of the invention as described hereinabove and as defined in the appended claims.

We claim:

1. A photographic silver halide emulsion desensitized to visible radiation with a thiuram disulfide silver halide desensitizer and a piazine containing a pyrazine ring to which two 6-membered carbocyclic rings are fused symmetrically.

2. A photographic silver halide emulsion desensitized to visible radiation with a thiuram disulfide silver halide desensitizer and a piazine having up to 24 carbon atoms and containing a pyrazine ring to which two 6-membered carbocyclic rings are fused symmetrically.

3. A photographic silver halide emulsion desensitized to visible radiation with a tetraalkyl thiuram disulfide silver halide desensitizer and a piazine having up to 24 carbon atoms and containing a pyrazine ring to which two 6-membered carbocyclic rings are fused symmetrically, the concentration of said thiuram disulfide being in the range of about 2 to about 75 mg. per mole of silver halide and the weight ratio of said thiuram disulfide to said piazine being in the range of about 2:1 to about 20:1.

4. A photographic silver halide emulsion desensitized to visible radiation with a tetraalkyl thiuram disulfide silver halide desensitizer and a piazine having the formula:



where each of R and R' is amino, hydroxy, hydrocarbyl amino, alkyl, aryl, acyloxy, acylamino or a fused 6-membered carbocyclic ring and each n is an integer of 0 to 2, the concentration of said thiuram disulfide being in the range of about 2 to about 75 mg. per mole of silver halide and the weight ratio of said thiuram disulfide to said piazine being in the range of about 2:1 to about 20:1.

5. A photographic silver halide emulsion desensitized to visible radiation with a tetraalkyl thiuram disulfide silver halide desensitizer and a piazine having the formula:



where each of R and R' is amino, hydroxy, hydrocarbyl amino, alkyl, aryl, acyloxy, acylamino or a fused 6-membered carbocyclic ring, R<sup>2</sup> is alkyl, hydroxyalkyl or aryl, X is an anion, each n is an integer of 0 to 2 and z is an integer of 0 to 1, the concentration of said thiuram disulfide being in the range of about 2 to about 75 mg.

bered carbocyclic ring, R<sup>2</sup> is alkyl, hydroxyalkyl or aryl, X is an anion, each n is an integer of 0 to 2 and z is an integer of 0 to 1, the concentration of said thiuram disulfide being in the range of about 2 to about 75 mg. per mole of silver halide and the weight ratio of said thiuram disulfide to said piazine being in the range of about 2:1 to about 20:1.

6. A photographic silver halide emulsion desensitized to visible radiation with bis(dimethylthiocarbamyl) disulfide and 1,3-diamino-5-methyl phenazinium chloride, the concentration of said disulfide being in the range of about 2 to about 75 mg. per mole of silver halide and the weight ratio of said disulfide to said phenazinium chloride being in the range of about 2:1 to about 20:1.

7. A photographic silver halide emulsion desensitized to visible radiation with bis(morpholinothiocarbamyl) disulfide and 1,3-diamino-5-methyl phenazinium chloride, the concentration of said disulfide being in the range of about 2 to about 75 mg. per mole of silver halide and the weight ratio of said disulfide to said phenazinium chloride being in the range of about 2:1 to about 20:1.

8. A photographic element comprising a support and a photographic silver halide emulsion layer desensitized to visible radiation with a thiuram disulfide silver halide desensitizer and a piazine containing a pyrazine ring to which two 6-membered carbocyclic rings are fused symmetrically.

9. A photographic element comprising a support and a photographic silver halide emulsion layer desensitized to visible radiation with a thiuram disulfide silver halide desensitizer and a piazine having up to 24 carbon atoms and containing a pyrazine ring to which two 6-membered carbocyclic rings are fused symmetrically.

10. A photographic element comprising a support and a photographic silver halide emulsion layer desensitized to visible radiation with a thiuram disulfide silver halide desensitizer and a piazine having up to 24 carbon atoms and containing a pyrazine ring to which two 6-membered carbocyclic rings are fused symmetrically, the concentration of said thiuram disulfide being in the range of about 2 to about 75 mg. per mole of silver halide and the weight ratio of said thiuram disulfide to said piazine being in the range of about 2:1 to about 20:1.

11. A photographic element comprising a support and a photographic silver halide emulsion layer desensitized to visible radiation with a tetraalkyl thiuram disulfide silver halide desensitizer and a piazine having the formula:



where each of R and R' is amino, hydroxy, hydrocarbyl amino, alkyl, aryl, acyloxy, acylamino or a fused 6-membered carbocyclic ring and each n is an integer of 0 to 2, the concentration of said thiuram disulfide being in the range of about 2 to about 75 mg. per mole of silver halide and the weight ratio of said thiuram disulfide to said piazine being in the range of about 2:1 to about 20:1.

12. A photographic element comprising a support and a photographic silver halide emulsion layer desensitized to visible radiation with a tetraalkyl thiuram disulfide silver halide desensitizer and a piazine having the formula:



where each of R and R' is amino, hydroxy, hydrocarbyl amino, alkyl, aryl, acyloxy, acylamino or a fused 6-membered carbocyclic ring, R<sup>2</sup> is alkyl, hydroxyalkyl or aryl, X is an anion, each n is an integer of 0 to 2 and z is an integer of 0 to 1, the concentration of said thiuram disulfide being in the range of about 2 to about 75 mg.

per mole of silver halide and the weight ratio of said thiuram disulfide to said piazine being in the range of about 2:1 to about 20:1.

13. A photographic element comprising a support and a photographic silver halide emulsion layer desensitized to visible radiation with bis(dimethylthio carbamyl) disulfide and 1,3-diamino-5-methyl phenazinium chloride, the concentration of said disulfide being in the range of about 2 to about 75 mg. per mole of silver halide and the weight ratio of said disulfide to said phenazinium chloride being in the range of about 2:1 to about 20:1.

14. A photographic element comprising a support and a photographic silver halide emulsion layer desensitized to visible radiation with bis(morpholinothio carbamyl) disulfide and 1,3-diamino-5-methyl phenazinium chloride, the concentration of said disulfide being in the range of about 2 to about 75 mg. per mole of silver halide and the weight ratio of said disulfide to said phenazinium chloride being in the range of about 2:1 to about 20:1.

15. A photographic silver halide desensitizing combination comprising a thiuram disulfide silver halide desensitizer and a piazine containing a pyrazine ring to which two 6-membered carbocyclic rings are fused symmetrically.

16. A photographic silver halide desensitizing combination comprising a thiuram disulfide silver halide desensitizer and a piazine having up to 24 carbon atoms and containing a pyrazine ring to which two 6-membered carbocyclic rings are fused symmetrically, the weight ratio of said thiuram disulfide to said piazine being in the range of about 5:1 to about 10:1.

17. A photographic silver halide desensitizing combination comprising a tetraalkyl thiuram disulfide silver halide desensitizer and a piazine having the formula:



where each of R and R' is amino, hydroxy, hydrocarbyl amino, alkyl, aryl, acyloxy, acylamino or a fused 6-membered carbocyclic ring and each n is an integer of 0 to 2, the weight ratio of said thiuram disulfide to said piazine being in the range of about 2:1 to about 20:1.

18. A photographic silver halide desensitizing combination comprising a tetraalkyl thiuram disulfide silver halide desensitizer and a piazine having the formula:



where each of R and R' is amino, hydroxy, hydrocarbyl amino, alkyl, aryl, acyloxy, acylamino or a fused 6-membered carbocyclic ring, R<sup>2</sup> is alkyl, hydroxyalkyl or aryl, X is an anion, each n is an integer of 0 to 2 and z is an integer of 0 to 1, the weight ratio of said thiuram disulfide to said piazine being in the range of about 2:1 to about 20:1.

19. A photographic silver halide desensitizing combination comprising bis(dimethylthio carbamyl) disulfide and 1,3-diamino-5-methyl phenazinium chloride, the weight ratio of said disulfide to said phenazinium chloride being in the range of about 2:1 to about 20:1.

20. A photographic silver halide desensitizing combination comprising bis(morpholinothio carbamyl) disulfide and 1,3-diamino-5-methyl phenazinium chloride, the weight ratio of said disulfide to said phenazinium chloride being in the range of about 2:1 to about 20:1.

35 No references cited.

NORMAN G. TORCHIN, Primary Examiner.

J. R. EVERETT, Assistant Examiner.